

[54] CARBON ANODE PROTECTION IN  
ALUMINUM SMELTING CELLS

[75] Inventors: William C. Sleppy, Belleville, Ill.;  
Ronald J. Campbell, Apollo, Pa.

[73] Assignee: Aluminum Company of America,  
Pittsburgh, Pa.

[22] Filed: June 28, 1973

[21] Appl. No.: 374,803

[52] U.S. Cl. .... 204/67

[51] Int. Cl. .... C22d 3/12

[58] Field of Search ..... 204/67

[56] References Cited

UNITED STATES PATENTS

2,947,673 8/1960 Sem et al. .... 204/67

|           |         |               |        |
|-----------|---------|---------------|--------|
| 2,464,267 | 3/1949  | Short .....   | 204/67 |
| 3,509,030 | 4/1970  | Gooding ..... | 204/67 |
| 3,696,008 | 10/1972 | Levitin ..... | 204/67 |

Primary Examiner—John H. Mack

Assistant Examiner—D. R. Valentine

Attorney, Agent, or Firm—Daniel A. Sullivan, Jr.

[57] ABSTRACT

In the operation of a cell for the electrolytic reduction of  $Al_2O_3$  dissolved in a cryolite bath of aluminum metal utilizing a carbon anode, the improvement wherein there is provided at the anode an atmosphere containing water in amounts effective for preventing anode dusting.

4 Claims, 2 Drawing Figures



PATENTED DEC 17 1974

3,855,086

SHEET 1 OF 2



**FIG. I**

PATENTED DEC 17 1974

3,855,086

SHEET 2 OF 2



FIG. 2

# CARBON ANODE PROTECTION IN ALUMINUM SMELTING CELLS

## BACKGROUND OF THE INVENTION

The present invention relates to the operation of aluminum reduction cells utilizing carbon anodes.

Depending upon operating conditions, consumption of carbon anodes in Hall-Heroult process cells ranges from one-third to three-quarters of a pound of carbon per pound of aluminum produced. The preferred conditions are those leading to the stoichiometric minimum consumption, 0.33 lbs. C/lb. Al, predicted by the net cell reaction:



In experiments on closing off the space above the electrolyte bath of a Hall-Heroult cell from the air, there has arisen an accumulation of carbon scum on the bath surface and a distribution of carbon dust throughout the electrolyte. This carbon scum and dust is caused by a deterioration of the carbon anodes. The phenomenon is referred to as anode dusting.

Carbon scum causes alumina feeding problems. The scum has made it impossible to replenish alumina consumed during electrolysis. As the dissolved alumina content of the bath decreases, scum formation accelerates. Carbon dust and scum increases the bath viscosity and hinders diffusion of oxygen-bearing ions to the anode, thus limiting anode current densities and affecting the heat balance of the cell. Increases in the viscosity and density of the bath lower the current efficiency and contribute to poor metal coalescence. The carbon in the scum and dust is not available for reaction with oxygen at the anode and so the gross consumption of carbon is increased by dusting. Because of carbon scum, the bath agitation supplied by anode bubble evolution is reduced and the tendency for electrolyte to solidify at the metal pad-bath interface increases. Ultimately, enough carbon dust can be distributed throughout the bath in closed cells to cause electronic conduction and complete loss of metal production. These conditions must be avoided for successful operation of an enclosed cell.

Prolonging the life of anodes will not only decrease carbon consumption, but in the case of pre-baked anodes will decrease the amount of anode butts to be recycled to the production of additional anodes and thereby decreases problems attendant upon evolution of fluorides during baking of anodes.

## SUMMARY OF THE INVENTION

In view of the above, it is an object of the present invention to provide a method for preventing the phenomenon of anode dusting, particularly in closed cells.

This, as well as other objects which will become apparent in the discussion that follows, are achieved, according to the present invention, by a process for producing aluminum wherein a carbon anode of a cell for the electrolytic reduction of  $\text{Al}_2\text{O}_3$  dissolved in a cryolite bath to aluminum metal is provided with an atmosphere containing water in amounts effective for preventing anode dusting.

## GENERAL ASPECTS OF THE INVENTION

It is believed that anode dusting is caused by atmolite

or sodium aluminum tetrafluoride,  $\text{NaAlF}_4$ , in vapor form. This substance attacks an anode and causes anode dusting.

Thus, in cell operation, a gaseous effluent containing gaseous fluorides is evolved from the electrolytic bath of alumina dissolved in molten cryolite (primarily cryolite or cryolite plus additional fluorides such as excess  $\text{AlF}_3$ ,  $\text{CaF}_2$ , and  $\text{LiF}$ ), and among such gaseous fluorides is atmolite.

Attack by atmolite on exposed carbon anode surfaces is particularly a problem when using closed cells, e.g. cells which are closed at the top by a plate.

The atmosphere containing water can be provided by surrounding anode surfaces located above the electrolytic bath with a skirt spaced from such surfaces, and injecting water vapor into the space between the skirt and the anode surfaces. Alternatively the water vapor can be provided by closing off a space above the electrolytic bath and dissolving in the electrolyte bath alumina containing enough water that sufficient water vapor is evolved and rises into the closed space to afford the desired protection. Such alumina can be produced by heating alumina trihydrate to the desired water content by well-known techniques; e.g. using rotary kilns. It is desirable to feed the alumina into the bath close to the anode or anodes.

It is believed that the amount of water vapor to be provided in an atmosphere around an anode surface depends to some extent on the amount of atmolite to be neutralized. In general, it is desirable to provide at least enough water vapor to react the atmolite stoichiometrically with the water vapor in accordance with the equation



## BRIEF DESCRIPTION OF THE DRAWINGS

FIG. 1 is an elevational, cross-sectional, broken-away view of a Soderberg anode type cell for use in the present invention.

FIG. 2 is a schematic representation, in cross-section, of bench-scale equipment for illustrating a part of the present invention.

## DESCRIPTION OF THE PREFERRED EMBODIMENTS

Preferably in the practice of the present invention,  $\text{Al}_2\text{O}_3$  is electrolytically decomposed to aluminum metal in an electrolyte bath between an anode and a cathodic interface formed between aluminum metal and the electrolyte bath, the bath consisting essentially of  $\text{Al}_2\text{O}_3$ ,  $\text{NaF}$ , and  $\text{AlF}_3$  and having a weight ratio  $\text{NaF}$  to  $\text{AlF}_3$  up to 1.1:1. The bath is maintained at an operating temperature greater than 40°C above the cryolite liquidus temperature of the bath and effective for preventing bath crusting in interfacial areas between the bath and aluminum metal. The cryolite liquidus temperature is that temperature at which cryolite first begins to crystallize on cooling the bath.

While the bath may consist only of  $\text{Al}_2\text{O}_3$ ,  $\text{NaF}$ ,  $\text{AlF}_3$ , it is possible to provide in the bath at least one halide compound of the alkali and alkaline earth metals other than sodium in an amount effective for reducing the liquidus temperature of the bath below that which it would have if only  $\text{Al}_2\text{O}_3$ ,  $\text{NaF}$ , and  $\text{AlF}_3$  were present. Suitable alkali and alkaline earth metal halides are  $\text{LiF}$ ,  $\text{CaF}_2$ , and  $\text{MgF}_2$ . In a preferred embodiment, the bath

contains lithium fluoride in an amount between 1 and 15 wt. %.

A preferred practice for maintaining the alumina concentration as electrolytic reduction proceeds is to add, substantially continuously, directly to the molten bath, an alumina which has a total water of 8 to 20 percent, more preferably 10 to 18 percent. The surface area may preferably be in the range 135 to 180 m<sup>2</sup>/g. The "total water" is a measure of the water in the alumina and is defined herein as follows:

Expose a sample of alumina to 100 percent humidity for several hours, then equilibrate the sample at 44 percent relative humidity, 25°C, for 18 hours, then accurately weigh the sample, then ignite it to 1,100°C, then weigh again. The loss in sample weight on going from the equilibrated state at 44 percent relative humidity to the ignited state after heating at 1,100°C, divided by the sample weight at 1,100°C, and multiplied by 100 is the percent total water.

Surface area is measured by the Brunauer-Emmett-Teller method. See Stephen Brunauer, P. H. Emmett, Edward Teller, *J. of Am. Chem. Soc.*, V. 60, Pgs. 309-19, 1938.

The use of alumina of the high water content of the present invention is contrary to the commonly-held view set forth at p. 34 of "The Chemical Background of the Aluminum Industry" by Pearson, published by The Royal Institute of Chemistry in 1955, that alumina used in electrolytic production of aluminum should be moisture-free.

Further illustrative of the present invention are the following examples:

#### EXAMPLE I

With reference to FIG. 2, there is shown a graphite crucible 51 having a non-conducting, refractory lining 52 with a hole 53 at its lower end. A molten aluminum metal pad 54 sits in the bottom of the alumina crucible and contacts the graphite crucible 52 to be in electrical contact with cathode lead 55. Resting on pad 54 is electrolyte bath 56 containing 4 wt. % Al<sub>2</sub>O<sub>3</sub> and NaF + AlF<sub>3</sub> at a bath weight ratio NaF/AlF<sub>3</sub> = 0.8. The electrolyte bath is at 900°C. Carbon (prebaked, petroleum coke) anode 57 is immersed in the electrolyte bath to provide an electrical current density of 5 amperes per inch<sup>2</sup> on the anode. Aluminum anode skirt 58 surrounds the anode 57 as shown and is sealed at its top by plug 59 provided with orifices for the passage of anode lead 60 and gas flow pipe 61. Appropriate piping is provided for allowing varied amounts of argon gas to flow from tank 62 through impinger bottle 63 containing water 64 surrounded by an ice water bath 65. Thus, the argon gas fed into the space between the anode 57 and the skirt 58 contained water vapor picked up by the argon from the water in the bottle 63. In operation of the cell to produce aluminum, carbon consumption was 0.33 to 0.38 pounds per pound of aluminum produced at a current efficiency of 100 percent in 29 to 41 ampere-hour tests using water vapor shielding for preventing anode dusting. With 4 to 22 torr water partial pressure in the argon, no carbon froth or scum was detected. When the impinger bottle 63 was bypassed so that only argon moved down around anode 57, a carbon scum formed on the surface of the bath 56, and electronic conduction through the carbon scum occurred.

#### EXAMPLES II AND III

Aluminum was produced in the cell of FIG. 1. The maximum dimensions of the steel shell 20 in the horizontal were 18' 6" × 10' 2". Its maximum height was 3' 9". The maximum dimensions of the molten aluminum metal pad 21 in the horizontal were 17' 8" × 9' 4". The electrolyte bath had the same maximum dimensions as the metal pad.

10 A mica mat 22 was provided between the steel shell 20 and graphite block 23 for the purpose of preventing current flow through shell 20. Mat thicknesses of from 6 to 20 mils have been used.

15 The pad 21 of molten aluminum was supported on carbonaceous cathode block lining 24 and carbonaceous tamped lining 25. The carbonaceous linings were supported on an alumina fill 26, there being interposed between the tamped lining and the fill some quarry tile 27. A layer of red brick 28 was provided between the graphite block 23 and quarry tile 27.

20 FIG. 1 is a representative vertical section through the cell and it will be realized that, for instance, similar graphite blocks 23 would appear in other elevational sections through the cell.

25 The anode 29 was a Soderberg-type carbon anode. The composition charged to form this self-baking anode was 31 percent pitch of softening point equals 98°-100°C (cube-in-air method) and 69 percent petroleum coke. The coke fraction was 30 percent coarse, 16 percent intermediate, and 54 percent fine, the size distributions of the coarse, intermediate, and fine coke being given in Table I.

Table I

| Tyler Sieve | Coke Size Distribution               |              |      |
|-------------|--------------------------------------|--------------|------|
|             | Cumulative % Greater Than Sieve Size |              |      |
|             | Coarse                               | Intermediate | Fine |
| .371        | 31.1                                 |              |      |
| 3           | 50.6                                 |              |      |
| 4           | 66.8                                 |              |      |
| 8           | 91.7                                 | 11           |      |
| 14          | 97.9                                 | 48.9         |      |
| 28          | 98.8                                 | 75.5         |      |
| 48          | 99.1                                 | 93.5         | 2.4  |
| 100         | 99.4                                 | 98.0         | 10.4 |
| 200         | 99.7                                 | 99.0         | 39.7 |
| pan         | 100                                  | 100          | 100  |

50 The cathode current was supplied through steel collector bars, such as bar 30, to the block lining 24. The current supply is indicated by the plus and minus signs on the anode and on collector bar 30 respectively.

55 The space above the bath 31 was sealed from the surrounding air by a closure 32, including a cast iron manifold 33, Ceraform Refractory board 34, which is a soft (for obtaining a good seal) fibrous electrical and heat insulating board available from the Johns-Manville Co., steel shell 35, steel plate 36, and fire clay brick, e.g. 50% Al<sub>2</sub>O<sub>3</sub> and 50% SiO<sub>2</sub>, 37. Within shell 35 there was provided a castable 38 serving a primarily insulative function and a castable 39, e.g. calcium-aluminate-bonded tabular alumina, selected for its refractory properties. The particular heat transfer situation was chosen to maintain the upper surface 45 of bath 31 substantially in molten condition, i.e. free of any crusting.

Alumina is charged from hopper 40 through a fill valve and feeder assembly 41 of the type disclosed in U.S. Pat. No. 3,681,229 issued Aug. 1, 1971 to R. L. Lowe entitled "Alumina Feeder." Measured quantities of alumina are fed onto the exposed molten bath surface through Inconel-600 pipe 42. The distance between the bottom of pipe 42 and the top of bath 31 is about 1 foot. The feeder 41 is a shot-type feeder, i.e. separate quantities of alumina are fed at timed intervals. In Examples II and III, two feeders 41 were used, and these fed-in alumina approximately every 5 minutes, the quantities of alumina being adjusted to maintain the desired alumina concentration in the bath. It takes about 1 minute to discharge the alumina increments which were about 1,500 grams. Pipe 42 is directed so as to impinge alumina onto the bath 31 where gas 44 is rising alongside the anode. This assures that the water evolved from the charged alumina protects the anode against production of carbon dust therefrom. This practice also promotes dissolution because of the bath agitation caused by the gas evolution. By charging the alumina in line with a spike row (spikes 45a, b, and c lie in a vertical plane parallel to the plane of FIG. 1, which plane also contains pipe 42) in the Soderberg anode (cracks usually occur in the anode in line with spike rows), the dissolution rate is enhanced by the additional gas evolution occurring at the cracks. Feeders 41 were operated using air as the fluidizing medium, it being recognized that this represents a small leakage of air past cover 32 to the bath.

The particular alumina used for Examples II and III had a total water of 16.95 percent. This alumina was 98 plus 325 mesh and its water content alone was sufficient to prevent anode dusting, i.e. a decomposition of the anode such that carbon particles build up in and on the bath.

The production data for Examples II and III are presented in Tables II to IV.

Table II

| Pot Production Data               |                   |                    |
|-----------------------------------|-------------------|--------------------|
| Data Name                         | Example No.<br>II | Example No.<br>III |
| Pot Days Operated                 | 32                | 96                 |
| Total Lbs. Net Aluminum (Al)      | 35,172            | 110,740            |
| Lbs. Net Al/Pot-Day               | 1099.2            | 1153.5             |
| Average % Al                      | 99.74             | 99.75              |
| Electrical Current Efficiency     | 92.6              | 90.0               |
| Kilowatt-Hours/Lb. of Al          | 7.49              | 7.76               |
| Anode Effects/Pot-Day             | .91               | 1.21               |
| Lbs. Soderberg Paste/Lb. Net Al   | .56               | N.M. <sup>1</sup>  |
| Lbs. Cryolite Used                | 1850              | 3600               |
| Lbs. Fluoride Used                | 6105              | 21,731             |
| Lbs. LiCO <sub>3</sub> Used       | 682               | 1400               |
| Anode to Cathode Distance, inches | 1.4               | 1.5                |

<sup>1</sup> N.M. = not measured

Table III

| Pot Electrical Data        |                   |                    |
|----------------------------|-------------------|--------------------|
| Data Name                  | Example No.<br>II | Example No.<br>III |
| Volts/Pot                  | 5.13              | 5.17               |
| Average Amperes            | 66,874            | 72,207             |
| Kilowatts/Pot              | 343.1             | 373.3              |
| Ohmic Voltage Drop in Bath | 1.70              | 1.68               |

Table IV

| Pot-Bath Data                                        |                   |                    |
|------------------------------------------------------|-------------------|--------------------|
| Data Name                                            | Example No.<br>II | Example No.<br>III |
| Wt.-% CaF <sub>2</sub>                               | 3.11              | 3.17               |
| Wt.-% Al <sub>2</sub> O <sub>3</sub>                 | 4.09              | 4.00               |
| Wt.-% AlF <sub>3</sub>                               | 48.97             | 45.08              |
| Wt.-% LiF                                            | 5.61              | 10.165             |
| Wt.-% NaF                                            | 38.13             | 36.94              |
| Wt.-% MgF <sub>2</sub>                               | .38               | .28                |
| Liquidus Temperature, °C                             | 882               | 906                |
| Calculated Wt.-Ratio NaF/AlF <sub>3</sub>            | .78               | .82                |
| Calculated Wt.-% Cryolite                            | 63.4              | 61.9               |
| Calculated Excess AlF <sub>3</sub>                   | 23.4              | 20.5               |
| Bath Operating Temperature, °C                       | 898               | 922                |
| "Eutectic" Temperature, °C                           | 799               | 814                |
| Conductivity, ohm <sup>-1</sup> inches <sup>-1</sup> | 4.87              | 5.67               |
| Bath Depth, inches                                   | 8.26              | 7.62               |
| Metal Depth, inches                                  | 6.02              | 6.25               |

With special reference to Table IV, the excess AlF<sub>3</sub> indicates the quantity of AlF<sub>3</sub> above that present under the heading cryolite, formula 3NaF.AlF<sub>3</sub>. In each of Examples II and III, Al<sub>2</sub>O<sub>3</sub> would be the first substance to crystallize on going below the given liquidus temperature. The "eutectic" temperature provides an estimate of the cryolite liquidus temperature in this case. The eutectic temperature is determined by finding the liquidus temperature for progressively decreasing Al<sub>2</sub>O<sub>3</sub> content, correspondingly increasing NaF + AlF<sub>3</sub>, and constant bath ratio NaF/AlF<sub>3</sub> and selecting the minimum liquidus temperature on the basis of the resulting group of liquidus temperature values. The Al<sub>2</sub>O<sub>3</sub> in solution is that at the particular bath operating temperature. Conductivity data is likewise for the given operating temperature.

Gases evolved from the Soderberg anode (e.g. hydrocarbons), fluorides from the bath, and anode reaction gas (e.g. CO<sub>2</sub>) were vented from cover 32 through an opening (not shown) and passed through a burner to burn the hydrocarbons. Because it is difficult to provide an absolute sealing of the bath from the air using cover 32, i.e. leaks can be present in cover 32, a pressure of 0.03 to 0.1 inch of H<sub>2</sub>O, measured negatively from atmospheric pressure, is maintained between the cover 32 and the burner, in order to prevent fume leakage from the cover 32. The burned gases were then fed to a scrubber system.

#### EXAMPLE IV

This Example illustrates how a suitable alumina product as used in Examples II and III can be produced.

Bayer-process alumina hydrate was treated in a kiln to produce kiln activated alumina suitable for use in the process of the present invention as follows. Kiln dimensions were 360 feet length and 9 1/2 feet inner-diameter. Residence time of the material in the kiln was 1 to 1 1/2 hours. The charged hydrate moved countercurrent to the combustion gases introduced into the lower end of the kiln. A maximum temperature of 400° to 500°C was achieved 10 to 15 feet inside the lower end of the kiln. Natural gas was burned at a rate of 6,500 cubic feet (standard temperature and pressure) per hour to produce the combustion gases. This natural gas flow rate was selected by testing the product for the desired total water. The volume ratio of air to gas was 10:1. An alumina having a 12.5 percent total water was produced. Anywhere from 88 to 95 weight % of the particles had a size greater than 325 mesh.

It will be understood that the above description of the present invention is susceptible to various modifications, changes, and adaptations and the same are intended to be comprehended within the meaning and range of equivalents of the appended claims.

It will likewise be recognized that the action of water in the present invention will be subject to energy-related laws such as rates of reaction and chemical equilibrium constants and that anode dusting need only be prevented to an extent such that there be no dusting-related impairment of cell operation.

All percentages given herein are in percent by weight unless indicated otherwise.

What is claimed is:

1. In the operation of a cell for the electrolytic reduction of  $\text{Al}_2\text{O}_3$  dissolved in a cryolite bath to aluminum metal utilizing a carbon anode, the improvement com- 15

prising providing at the anode an atmosphere containing water in amounts effective for preventing anode dusting.

2. In the operation of a cell as claimed in claim 1, the improvement further being characterized by a closing of the top of the cell.

3. In the operation of a cell as claimed in claim 1, the improvement being further characterized by the providing of a skirt around the anode, said atmosphere 10 being provided within said skirt.

4. In the operation of a cell as claimed in claim 1, the improvement being further characterized in that the amount of water is at least enough for reacting atomolite stoichiometrically according to the equation



\* \* \* \* \*

20

25

30

35

40

45

50

55

60

65

UNITED STATES PATENT OFFICE  
CERTIFICATE OF CORRECTION

Patent No. 3,855,086 Dated December 17, 1974

Inventor(s) William C. Sleppy et al

It is certified that error appears in the above-identified patent and that said Letters Patent are hereby corrected as shown below:

In the Abstract,  
line 2

After "bath" change "of"  
to --to--.

Signed and sealed this 11th day of February 1975.

(SEAL)  
Attest:

RUTH C. MASON  
Attesting Officer

C. MARSHALL DANN  
Commissioner of Patents  
and Trademarks